

Nov. 24, 1953

H. S. HILL

2,660,097

METHOD OF PROCESSING WOOD PULP

Filed April 16, 1949



INVENTOR.  
HAROLD S. HILL

BY

*B. Shlesinger*

ATTORNEY

## UNITED STATES PATENT OFFICE

2,660,097

## METHOD OF PROCESSING WOOD PULP

Harold Sanford Hill, Kenogami, Quebec, Canada,  
assignor to Price Brothers & Company, Lim-  
ited, Quebec, Canada, a corporation of Quebec,  
Canada

Application April 16, 1949, Serial No. 87,893

4 Claims. (Cl. 92—20)

1

The present invention relates to the mechanical processing of pulp for papermaking. More particularly the invention relates to the mechanical processing of chemical pulps, such as sulphite pulps, by the pulp treating method disclosed in the pending U. S. patent application of the present inventor and Joseph Edwards, Serial No. 565,128, filed November 25, 1944, which has now matured into Patent No. 2,516,384, granted July 25, 1950.

In the process of Patent No. 2,516,384, the pulp, which is to be treated, is brought to a state in which its mass is made up of small, discrete nodules moist with an aqueous liquid; a layer of the nodulated pulp is compressed between two working surfaces, which are roughened or figured to have good traction with the pulp without entangling the fibres; and the nodulated pulp is caused to roll tractively in traverse of and under compression by the surfaces in such way that the nodules are continuously or frequently re-oriented with reference to the direction in which the nodulated pulp rolls in traverse of the surfaces. The reorientation of the nodules may be effected in various ways. A preferred method is by causing the direction in which the nodulated pulp rolls in traverse of the surfaces to change continuously with reference to the surfaces along curved paths. A preferred way of accomplishing this continuous change in direction of roll of the nodulated pulp over the surfaces is to impart to one of the surfaces a circulatory translatory motion so that each point on the surface moves in a separate circular path. This is in contradistinction to a simple rotary motion in which all points of the rotary surface revolve about a common axis.

The process of Patent No. 2,516,384 imparts new and valuable properties to papermaking pulp, and, in addition, exerts a very powerful defibring action on any shives or fibre bundles which may be present in the pulp. Among the important applications of the process of the patent mentioned has been that of treating high-yield chemical pulp.

One of the fundamental requirements for carrying out the process of Patent No. 2,516,384 is that true rolling traction of the pulp on the working surfaces be maintained at all times. The pulp must not slip on the surfaces; and slip or shear planes must not be allowed to develop within the pulp itself. If such slippage occurs, or if shear planes develop within the pulp, the rolling traverse of the pulp over the working surfaces ceases at once; the pulp forms into

2

matted sliding layers; and the functioning of the process as such comes to a complete stop.

It has been found that slippage occurs and shear planes develop if the rolling traverse of the pulp over the surfaces exceeds a critical velocity, and further, if the compression of the pulp during rolling exceeds a critical pressure. The two factors, velocity of rolling and pressure, are to a considerable extent interdependent, the lower the velocity, the high the pressure that can be employed without loss of traction and vice versa. In practice, the speed of relative movement of the working surfaces is usually in the range of 100 to 300 feet per minute, and the pressure exerted on the pulp by the surfaces is usually in the range of 5 to 20 pounds per square inch of opposed surfaces compressing the pulp.

It will be apparent that the velocity of rolling and the applied pressure combine to provide a measure of the power input, and that since there are definite limits to both velocity and pressure in carrying out the process, it follows, in turn, that there is a definite limit to the intensity of power input that may be used. This is a factor of great importance in the practical application of the process of Patent No. 2,516,384 since it imposes a limit on the work that can be obtained from a given area of working surfaces; in short, it puts a limit on the capacity of a given processing machine.

As far as is known, this ability of a pulp to absorb power in rolling under compression is one that, prior to the invention of the process of Patent No. 2,516,384, had received no recognition or interest. Indeed, it is a property of pulp which as yet has been given no name in the art. For the purpose of the present application this property is designated as "traction." A pulp, which has marked ability to absorb power when treated by the process of Patent No. 2,516,384, is said to possess high traction; a pulp, which has poor ability to absorb power when treated by such process, is said to possess low traction. Various kinds and grades of chemical pulps exhibit different amounts of traction. High-yield sulphite pulps have relatively low traction, and, in general, the traction becomes less and less with increasing yield.

A primary object of the present invention is to improve the traction of chemical papermaking pulp so that it may readily be processed by the method of Patent No. 2,516,384.

Another object of the invention is to improve the efficiency of the method of Patent No. 2,516,384 in the treatment of chemical pulp.

Still another object of the invention is to provide an improved method of preparing a low-cost furnish in the manufacture of newsprint paper.

Other objects of the invention will be apparent hereinafter from the specification and from the recital of the appended claims.

I have found that the traction of a chemical pulp may be raised to a notable degree by incorporating with the chemical pulp some ground wood. By groundwood is meant the well known pulp made by pressing wood against the face of a revolving grindstone.

In the method of the present application a minor fraction of groundwood is added to the chemical pulp prior to mechanical processing. An example will serve to illustrate the remarkable improvement in operating efficiency that may be achieved by this method. In an installation for carrying out the process of Patent No. 2,516,384 using a machine of suitable type a high-yield sulphite pulp was being processed at the rate of about 17 tons per day. The pulp was of the low traction variety and the machine capacity was limited to the above figure at a given pulp temperature because if either the speed of surface movement or the operating pressure were increased, slipping of the pulp would occur and it would smear and build up on the working surfaces. By adding 10% of groundwood to the high-yield sulphite prior to processing, the capacity of the machine in doing the same work on the pulp was raised to 35 to 40 tons per day. This added loading of the machine could be accomplished either by increasing the speed of surface movement or increasing the operating pressure of the surfaces on the pulp. The ability of the high-yield sulphite to absorb power without slipping was thus greatly increased by the addition of groundwood. In terms of efficiency, with the added groundwood, then, one machine could handle a production tonnage which otherwise would have required two machines. There are other advantages, also, to the addition of groundwood. With the addition of the groundwood it was possible to operate at a lower stock temperature and thus save steam.

Addition of groundwood not only makes it possible to obtain better operating efficiency in the treatment of high-yield pulps, but also renders some high-yield pulps processable which could not be treated at any practical rate by the process of Patent No. 2,516,384. Some high-yield pulps are so slippery that normally it has not been practical heretofore to treat them by the process of Patent No. 2,516,384. With the addition of a minor fraction of groundwood, however, they may readily be treated by this process at good efficiency.

The groundwood may be added to the chemical pulp at any convenient point prior to processing the chemical pulp by the method of Patent No. 2,516,384, and in any convenient way. In continuous process it is of course preferable that the groundwood be added at a uniform, controlled rate. The amount of groundwood, which is used, may vary over a considerable range depending on the operating requirements in a particular case. In some instances 3% of groundwood added to the chemical pulp will provide the desired improvement in operating efficiency, while with some very low traction pulps 25% or even higher of groundwood addition may be required.

I have found further that the method of the

present invention may serve as a key part of a novel system of preparing furnish for newsprint manufacture which will permit an efficiency and a low cost hitherto unobtainable. In the conventional method of preparing newsprint furnish, sulphite pulp cooked in the digesters to give about 47 percent yield on the wood is screened and then mixed at the regulators in predetermined proportion with groundwood pulp made at the grinders and then screened. The mixture, including any desired coloring matter, is then passed to the paper machine. The proportion of sulphite pulp in the furnish is usually in the range of 12% to 20%. In some cases, a portion of mineral loading material is added before or at the paper machine.

In the accompanying drawing:

Fig. 1 is a flow sheet illustrating diagrammatically one way in which an improved, low cost newsprint furnish may be prepared by the method of the present invention.

In my novel system of preparing newsprint furnish, the groundwood may be made in the usual way, but the sulphite pulp may be made to have a higher yield on the basis of the wood used in the range of 55 to 75%, the increased yield being obtained by the use of milder cooking conditions at the digester, as is well known in the art. The groundwood passes, of course, from the pulp grinding station to the screening station where the usual screening operations are carried out to eliminate oversize material.

With the method of the present invention, a small portion of the screened groundwood, usually in the range of 0.5% to 8% of the total amount of groundwood, is bypassed and mixed with the unrefined high-yield sulphite pulp coming from the digester, the proportion being usually in the range of 3% to 40% groundwood to 97% to 60% of high-yield sulphite. The mixture of the two pulps is then passed to a refiner of suitable type operating according to the process of application Serial No. 565,128, and in this machine the mixed pulp is brought to a state in which its mass is made up of small, moist, discrete nodules, usually of a consistency in the order of about 20%, and the nodules are rolled tractively between and in traverse of two opposed working surfaces which compress the nodules while they roll, the rolling motion being effected by moving the upper working surface bodily with a circular gyratory or translatory motion about an axis extending in the direction of applied pressure. Thus, the compressed nodulated pulp is rolled over the working surfaces in continuously changing directions, and the individual fibers are thereby given innumerable short-radius, flexing actions. This treatment changes the harsh, shiv, high-yield pulp to a well defibered pulp of a softened character particularly suited to the requirements of newsprint manufacture and quality. Due to the presence of the groundwood, the refiner can operate at high capacity and efficiency.

The processed, mixed pulp from the refiner is then put through the usual screening operation, as illustrated in Fig. 1. A pulp washing step may be included if desired. The screened mixture is then mixed in regulated amount with the main, untreated groundwood which represents usually 92% to 99.5% of the total amount of groundwood used. The combined pulps, namely, the mixture of untreated groundwood and of the refined mixture of chemical pulp and groundwood constitutes the furnish, and are then delivered

to the papermaking machine for treatment in the usual way.

Fig. 1 shows diagrammatically the above described steps in the preparation of the newsprint furnish as applied in an integrated pulp and newsprint manufacturing operation.

While the invention has particular application to the processing of pulp by the method of Patent No. 2,516,384, it may also be used with advantage in other mechanical processes for refining pulp. While a particular embodiment of the invention and a particular use therefor have been described, then, it will be understood that the invention is capable of further modification and use, and this application is intended to cover any variations, uses, or adaptations of the invention following, in general, the principles of the invention and including such departures from the present disclosure as come within known or customary practice in the art to which the invention pertains and as may be applied to the essential features hereinbefore set forth and as fall within the scope of the invention or the limits of the appended claims.

Having thus described my invention, what I claim is:

1. The method of preparing a papermaking furnish made up of 10% to 25% raw chemical wood pulp as one component and of 90% to 75% of groundwood as another component, which includes as one step the rolling of moist, nodulated pulp tractively in traverse of and under compression by and between two opposed working surfaces, which comprises first mixing 0.5% to 8% of the groundwood with the raw chemical pulp, thereby to increase the ability of the pulp to absorb working power without slipping or smearing on the working surfaces, bringing the mixture to a state in which its mass is made up of small, moist, discrete nodules of fibres at high consistency, compressing the nodulated mixture between two opposed working surfaces which are roughened to provide traction for the pulp without obstructing rolling traverse of the pulp nodules on said surfaces, rolling the nodulated mixture tractively in traverse of the working surfaces while it is under compression between them to refine the mixture, and then mixing the balance of the groundwood component of the furnish with the refined mixture.

2. The method of processing a slippery, moist chemical pulp which comprises increasing the ability of the pulp to absorb working power without slipping by adding to the moist chemical pulp a minor proportion of groundwood prior to refining the pulp, and then refining the pulp by forming the mixture of pulp and groundwood into small, moist, discrete nodules, comprises the mixture while in a moist nodulated state between two opposed working surfaces which are roughened to provide traction for the pulp without obstructing rolling traverse of the pulp nodules on the working surfaces, and rolling the nodulated mixture tractively in traverse of and under compression between the two opposed working surfaces.

3. The method of utilizing a slippery, raw, high-yield, chemical pulp in newsprint furnish which comprises adding to the slippery, raw pulp

a minor proportion of groundwood, thereby to increase substantially the ability of the pulp to absorb working power without slipping when the raw pulp is refined by causing it to roll in moist, nodule form under compression between opposed working surfaces, forming the mixture of raw pulp and groundwood to a state of small, discrete, moist nodules, compressing the nodulated pulp between two opposed working surfaces which are roughened to have tractive contact with the pulp without obstructing rolling traverse of the pulp nodules on the surfaces, causing the compressed, nodulated mixture to roll under compression between and across the two opposed working surfaces to refine it, and then adding to the refined mixture an additional major proportion of groundwood to form newsprint furnish.

4. The method of producing a papermaking furnish from a high-yield, raw, chemical pulp, which comprises first mixing a minor proportion of groundwood with a moist, raw, high-yield chemical pulp, thereby to increase the ability of the pulp to absorb working power without slipping or smearing when rolled between opposed working surfaces, forming the mixture into small, discrete, moist nodules, compressing the nodules between two opposed working surfaces which are roughened to provide traction for the pulp without obstructing rolling traverse of the pulp nodules on the two working surfaces, and rolling the pulp on and across the two working surfaces while under compression to refine the mixture, and then mixing additional groundwood with the refined mixture to form the furnish, the percentage of chemical pulp in the furnish being less than the percentage of the total amount of groundwood employed but being greater than the percentage of groundwood which is mixed with the chemical pulp before refining.

HAROLD SANFORD HILL.

References Cited in the file of this patent

UNITED STATES PATENTS

| Number    | Name                 | Date           |
|-----------|----------------------|----------------|
| 145,620   | Brown et al. -----   | Dec. 16, 1873  |
| 487,913   | Carter et al. -----  | Dec. 13, 1892  |
| 657,206   | Ferrell et al. ----- | Sept. 4, 1900  |
| 693,941   | Zilles -----         | Feb. 25, 1902  |
| 1,372,640 | Clapp -----          | Mar. 22, 1921  |
| 1,525,050 | Savery -----         | Feb. 3, 1925   |
| 1,757,010 | Fair -----           | May 6, 1930    |
| 1,881,419 | Munroe -----         | Oct. 4, 1932   |
| 2,214,893 | Von Hassell -----    | Sept. 17, 1940 |
| 2,456,249 | Bidwell -----        | Dec. 14, 1948  |
| 2,503,454 | Quinn -----          | Apr. 11, 1950  |
| 2,516,384 | Hill et al. -----    | July 25, 1950  |
| 2,573,709 | Hill et al. -----    | Nov. 6, 1951   |
| 2,580,161 | Driessen -----       | Dec. 25, 1951  |

OTHER REFERENCES

Modern Pulp and Paper Making Witham, 1942, 2nd ed., Reinhold Publishing Corp., page 72.

Deinking of Paper by West, page 10, (1943), published by Institute of Paper Chemistry, Appleton, Wisconsin.

Pulp and Paper Mag. of Canada, vol. 50, No. 3, pp. 153-160, 191, and 195-200 (1949).